



US010141099B2

(12) **United States Patent**  
**Jeong**

(10) **Patent No.:** **US 10,141,099 B2**  
(45) **Date of Patent:** **Nov. 27, 2018**

(54) **ELECTRONIC COMPONENT AND  
MANUFACTURING METHOD THEREOF**

(71) **Applicant:** **SAMSUNG  
ELECTRO-MECHANICS CO., LTD.,**  
Suwon-Si, Gyeonggi-Do (KR)

(72) **Inventor:** **Dong Jin Jeong**, Suwon-Si (KR)

(73) **Assignee:** **SAMSUNG  
ELECTRO-MECHANICS CO., LTD.,**  
Suwon-si, Gyeonggi-Do (KR)

(\*) **Notice:** Subject to any disclaimer, the term of this  
patent is extended or adjusted under 35  
U.S.C. 154(b) by 0 days.

(21) **Appl. No.:** **14/939,765**

(22) **Filed:** **Nov. 12, 2015**

(65) **Prior Publication Data**

US 2016/0217907 A1 Jul. 28, 2016

(30) **Foreign Application Priority Data**

Jan. 28, 2015 (KR) ..... 10-2015-0013602

(51) **Int. Cl.**

**H01F 5/00** (2006.01)  
**H01F 27/28** (2006.01)  
**H01F 7/06** (2006.01)  
**H01F 27/29** (2006.01)  
**H01F 17/00** (2006.01)  
**H01F 41/04** (2006.01)  
**H01F 17/04** (2006.01)

(52) **U.S. Cl.**

CPC ..... **H01F 27/292** (2013.01); **H01F 17/0013**  
(2013.01); **H01F 41/042** (2013.01); **H01F  
2017/048** (2013.01)

(58) **Field of Classification Search**

CPC .. H01F 27/2804; H01F 27/255; H01F 27/292;  
H01F 14/0013; H01F 14/0006; H01F  
2017/048; H01F 41/041; H01F 41/0233;  
H01F 2017/0073  
USPC ..... 336/200, 223, 233, 234; 29/602.1, 605,  
29/606

See application file for complete search history.

(56) **References Cited**

U.S. PATENT DOCUMENTS

7,759,776 B2 7/2010 Cheng  
2004/0056749 A1\* 3/2004 Kahlmann ..... H01L 27/08  
336/200

(Continued)

FOREIGN PATENT DOCUMENTS

CN 101046482 A 10/2007  
CN 101620916 A 1/2010

(Continued)

OTHER PUBLICATIONS

Chinese Office Action dated May 18, 2017, issued in Chinese Patent  
Application No. 201510849783.5. (w/ English translation).

(Continued)

*Primary Examiner* — Mangtin Lian

(74) *Attorney, Agent, or Firm* — McDermott Will &  
Emery LLP

(57) **ABSTRACT**

An electronic component includes a magnetic body and an internal coil structure embedded in the magnetic body. The internal coil structure includes a first coil pattern part and a second coil pattern part formed on the first coil pattern part. An outermost coil pattern portion of the first coil pattern part is thicker than an inner coil pattern portion thereof.

**20 Claims, 4 Drawing Sheets**



(56)

## References Cited

## U.S. PATENT DOCUMENTS

- 2004/0164835 A1\* 8/2004 Shoji ..... H01F 17/0013  
336/200  
2007/0235873 A1\* 10/2007 Cheng ..... G01R 1/07378  
257/738  
2008/0174397 A1\* 7/2008 de Rooij ..... G01R 33/34  
336/200  
2009/0322458 A1\* 12/2009 Lee ..... H01F 17/0006  
335/299  
2013/0249662 A1\* 9/2013 Tonoyama ..... H01F 27/255  
336/200  
2013/0300529 A1 11/2013 Chang et al.  
2013/0335186 A1\* 12/2013 Chang ..... H01F 5/003  
336/200  
2014/0197917 A1 7/2014 Naito et al.  
2015/0035640 A1\* 2/2015 Wang ..... H01F 17/0006  
336/200  
2015/0123757 A1 5/2015 Choi

## FOREIGN PATENT DOCUMENTS

- CN 103377811 A 10/2013  
CN 103733280 A 4/2014  
CN 104282421 A 1/2015  
EP 2645385 A2 10/2013  
JP 10-241983 A 9/1997  
JP 2001-267166 A 9/2001  
JP 2004-319570 A 11/2004  
JP 2006-278479 A 10/2006  
JP 2010016337 A 1/2010  
KR 101474166 B1 12/2014

## OTHER PUBLICATIONS

Korean Office Action issued in Korean Patent Application No. 10-2015-0013602, dated Jun. 16, 2017.

\* cited by examiner



FIG. 1



FIG. 2

FIG. 3



'A'

FIG. 4



'A'



FIG. 5

## 1

ELECTRONIC COMPONENT AND  
MANUFACTURING METHOD THEREOFCROSS-REFERENCE TO RELATED  
APPLICATION

This application claims benefit of priority to Korean Patent Application No. 10-2015-0013602 filed on Jan. 28, 2015, with the Korean Intellectual Property Office, the disclosure of which is incorporated herein in its entirety by reference.

## TECHNICAL FIELD

The present disclosure relates to an electronic component and a manufacturing method thereof.

## BACKGROUND

An inductor, an electronic component, is a representative passive element configuring an electronic circuit together with a resistor and a capacitor, to remove noise therefrom.

A thin film inductor is commonly manufactured by forming a coil pattern by plating and then hardening a magnetic powder-resin composite in which a magnetic powder and a resin are mixed with each other to form a magnetic body, and forming external electrodes on outer surfaces of the magnetic body.

In accordance with recent trends for increased complexity, slimness, multifunctionality and the like, in device components, attempts at manufacturing a thin film inductor having a reduced thickness have continued. Therefore, thin film inductors allowing high performance and reliability to be secured therein, even in light of the trend for device component slimness are required.

## SUMMARY

An aspect of the present disclosure may provide a slim electronic component having improved electrical properties by controlling a thickness of a first coil pattern part to induce anisotropic plating growth of a second coil pattern part, and a method for effectively manufacturing the electronic component.

According to an aspect of the present disclosure, an electronic component may include a magnetic body and an internal coil structure embedded in the magnetic body. The internal coil structure may include a first coil pattern part and a second coil pattern part formed on the first coil pattern part. An outermost coil pattern portion of the first coil pattern part may be thicker than an inner coil pattern portion thereof.

When a thickness of the outermost coil pattern portion of the first coil pattern part is a and a thickness of the inner coil pattern portion thereof is b,  $0 \mu\text{m} < a - b \leq 20 \mu\text{m}$  may be satisfied.

When a thickness of the outermost coil pattern portion of the first coil pattern part is a and a thickness of the inner coil pattern portion thereof is b,  $1 < a/b \leq 1.8$  may be satisfied.

A difference between a sum of a thickness of the outermost coil pattern portion of the first coil pattern part and a thickness of an outermost coil pattern portion of the second coil pattern part formed thereon and a sum of a thickness of the inner coil pattern portion of the first coil pattern part and a thickness of an inner coil pattern portion of the second coil pattern part formed thereon may be within 20  $\mu\text{m}$ .

The second coil pattern part may be formed by anisotropic plating.

## 2

The second coil pattern part may be formed on upper surfaces of the coil pattern portions of the first coil pattern part.

The second coil pattern part may not be formed on at least a portion of side surfaces of the coil pattern portions of the first coil pattern part.

The first and second coil pattern parts may be formed of the same metal.

The magnetic body may contain a magnetic metal powder and a thermosetting resin.

The internal coil structure may include a first internal coil structure disposed on one surface of a support member and a second internal coil structure disposed on the other surface of the support member opposing one surface thereof.

The support member may have a through-hole in a central portion thereof, and the through-hole may be filled with a magnetic material to form a core part.

The electronic component may further include external electrodes disposed on outer surfaces of the magnetic body to be electrically connected to the internal coil structure.

According to another aspect of the present disclosure, a method of manufacturing an electronic component may include forming an internal coil structure on a support member and forming a magnetic body by stacking magnetic sheets to embed the internal coil structure therein. The internal coil structure may include a first coil pattern part formed on the support member and a second coil pattern part formed on the first coil pattern part. An outermost coil pattern portion of the first coil pattern part may be thicker than an inner coil pattern portion thereof.

The method may further include forming external electrodes on outer surfaces of the magnetic body to be electrically connected to the internal coil structure.

The second coil pattern part may be formed by anisotropic plating.

## BRIEF DESCRIPTION OF DRAWINGS

The above and other aspects, features and advantages of the present disclosure will be more clearly understood from the following detailed description taken in conjunction with the accompanying drawings.

FIG. 1 is a perspective view schematically illustrating an electronic component including internal coil structures according to an exemplary embodiment in the present disclosure.

FIG. 2 is a cross-sectional view taken along line I-I' of FIG. 1.

FIG. 3 is an enlarged view schematically illustrating an example of part 'A' of FIG. 2.

FIG. 4 is an enlarged view schematically illustrating another example of part 'A' of FIG. 2.

FIG. 5 is a flowchart illustrating a method of manufacturing an electronic component according to an exemplary embodiment in the present disclosure.

## DETAILED DESCRIPTION

Hereinafter, embodiments of the present disclosure will be described in detail with reference to the accompanying drawings.

The disclosure may, however, be embodied in many different forms and should not be construed as being limited to the embodiments set forth herein. Rather, these embodiments are provided so that this disclosure will be thorough and complete, and will fully convey the scope of the disclosure to those skilled in the art.

In the drawings, the shapes and dimensions of elements may be exaggerated for clarity, and the same reference numerals will be used throughout to designate the same or like elements.

### Electronic Component

Hereinafter, an electronic component, particularly, a thin film inductor, according to an exemplary embodiment, will be described. However, the electronic component according to exemplary embodiments is not necessarily limited thereto.

FIG. 1 is a schematic perspective view illustrating an electronic component including internal coil structures according to an exemplary embodiment in the present disclosure. Referring to FIG. 1, as an example of the electronic component, a thin film inductor used for a power line of a power supply circuit is disclosed.

The electronic component 100 according to an exemplary embodiment may include a magnetic body 50, internal coil structures 41 and 42 embedded in the magnetic body 50, and first and second external electrodes 81 and 82 disposed on outer surfaces of the magnetic body 50 to be electrically connected to the internal coil structures 41 and 42.

In the electronic component 100 according to an exemplary embodiment, a 'length' direction refers to an 'L' direction of FIG. 1, a 'width' direction refers to a 'W' direction of FIG. 1, and a 'thickness' direction refers to a 'T' direction of FIG. 1.

The magnetic body 50 may form the exterior of the electronic component 100, and may be formed by including ferrite or magnetic metal particles in a resin part. However, a material for forming the magnetic body is not specifically limited, as long as the material exhibits magnetic properties.

Specific examples of the ferrite may include Mn—Zn-based ferrite, Ni—Zn-based ferrite, Ni—Zn—Cu-based ferrite, Mn—Mg-based ferrite, Ba-based ferrite, or Li-based ferrite. The magnetic body (50) may have ferrite particles dispersed in a resin such as epoxy or polyimide.

In addition, the magnetic metal particles may include at least one selected from the group consisting of Fe, Si, Cr, Al and Ni. For example, the magnetic metal particles may be a Fe—Si—B—Cr-based amorphous metal, but examples of the magnetic metal particles are not necessarily limited thereto. The magnetic metal particles may have a diameter of about 0.1  $\mu\text{m}$  to 30  $\mu\text{m}$ , and similar to the above-described ferrite, the magnetic body 50 may have the magnetic metal particles dispersed in a thermosetting resin such as epoxy or polyimide.

The first internal coil structure 41 having a coil shape may be disposed on one surface of a support member 20 disposed in the magnetic body 50, and the second internal coil structure 42 having a coil shape may be disposed on the other surface of the support member 20 opposing the one surface of the support member 20. In this case, the first and second internal coil structures 41 and 42 may be electrically connected to each other by a via 45 formed by filling a via hole penetrating through the support member 20 with a conductive material. The first and second internal coil structures 41 and 42 may have a spiral shape.

For example, the support member 20 may be a polypropylene glycol (PPG) substrate, a ferrite substrate or a metallic soft magnetic substrate, and the like. The support member 20 may have a through-hole penetrating through the central portion thereof, and the through-hole may be filled with a magnetic material to form a core part 55. The core part 55

made of the magnetic material may be formed as described above to improve performance of the thin film inductor.

The first and second internal coil structures 41 and 42 and the via 45 may contain a metal having excellent electrical conductivity, and for example, may be formed of silver (Ag), palladium (Pd), aluminum (Al), nickel (Ni), titanium (Ti), gold (Au), copper (Cu), platinum (Pt), alloys thereof, and the like. In this case, the first and second internal coil structures 41 and 42 having a thin film shape may be formed by electroplating, but may be formed by other methods known in the art as long as the first and second internal coil structures having a thin film shape are formed.

Meanwhile, direct current resistance  $R_{dc}$ , one of the main characteristics of the inductor, is decreased as cross-sectional areas of the internal coil structures are increased. In addition, inductance of the inductor is increased as an area of a magnetic body through which magnetic flux passes is increased. Therefore, in order to decrease direct current resistance  $R_{dc}$  and increase inductance, the cross-sectional areas of the internal coil structures need to be increased and the area of the magnetic body needs to be increased.

Increasing widths of coil pattern portions and increasing thicknesses of the coil pattern portions may increase the cross-sectional areas of the internal coil structures. However, when the widths of the coil pattern portions are increased, a possibility of short-circuits occurring between the coil pattern portions may be excessively increased, the number of turns of a coil may be limited, and an area of the magnetic body may be decreased, such that efficiency may be deteriorated and there may be limitations in implementing a product having high inductance.

Accordingly, the internal coil structures having a high aspect ratio (AR) by increasing thicknesses of the coil pattern portions without increasing widths of the coil pattern portions are required. Here, the aspect ratio (AR) of the internal coil structures refers to a value obtained by dividing the thickness of a coil pattern portion by the width of the coil pattern portion. As an increased amount of the thickness of the coil pattern portion is larger than an increased amount of the width of the coil pattern portion, the high aspect ratio (AR) may be implemented.

However, as plating proceeds during electroplating, due to isotropic growth in width and thickness directions, short-circuits may occur between the coil pattern portions, and thus, it may be difficult to implement internal coil structures having a high aspect ratio (AR).

According to an exemplary embodiment, the shape of coil pattern parts of the internal coil structures may be controlled to induce anisotropic plating growth as described below, thereby forming internal coil structures having a high aspect ratio (AR).

FIG. 2 is a cross-sectional view taken along line I-I' of FIG. 1. FIG. 3 is an enlarged view schematically illustrating an example of part 'A' of FIG. 2. Referring to FIGS. 2 and 55 3, the first and second internal coil structures 41 and 42 may include a first coil pattern part 61 formed on the support member 20, and a second coil pattern part 62 formed on the first coil pattern part 61.

In the first coil pattern part 61 according to an exemplary embodiment, an outermost coil pattern portion 61c may be thicker than inner coil pattern portions 61a and 61b, and in this case, a final thickness  $d$  of the internal coil structure (the coil pattern) formed by inducing anisotropic plating growth may be uniform. On the contrary, when the thickness of the outermost coil pattern portion 61c of the first coil pattern part 61 is equal to or thinner than that of the inner coil pattern portions 61a and 61b thereof, the final thickness  $d$  of

the coil pattern formed by anisotropic plating may be non-uniform, and therefore, short-circuits may occur between the coil pattern portions. Meanwhile, although the inner coil pattern portions **61a** and **61b** having the same thicknesses are illustrated in the drawings, the thicknesses of the inner coil pattern portions may not be necessarily equal to each other so long as the inner coil pattern portions **61a** and **61b** are thinner than the outermost coil pattern portion **61c**.

When the thickness of the outermost coil pattern portion **61c** is  $a$  and the thickness of the inner coil pattern portions **61a** and **61b** is  $b$ , Equation (1) below may be satisfied. When the thickness of the outermost coil pattern portion **61c** and the thickness of the inner coil pattern portions **61a** and **61b** satisfy Equation (1) below, the final thickness  $d$  of the coil pattern formed by inducing anisotropic plating growth may be uniform, and as a result, the electronic component may have unexpectedly excellent electrical performance. Meanwhile, when a difference between the thickness of the outermost coil pattern portion **61c** and the thickness of the inner coil pattern portions **61a** and **61b** is greater than  $20 \mu\text{m}$ , short-circuits may occur among the coil pattern portions due to overgrowth of the outermost coil pattern portion **61c**. Meanwhile, in Equation (1) below,  $0 \mu\text{m} < a - b < 20 \mu\text{m}$  may be satisfied, but the range of  $a - b$  is not limited thereto:

$$0 \mu\text{m} < a - b \leq 20 \mu\text{m}.$$

Equation (1)

Similar to the above description, when the thickness of the outermost coil pattern portion **61c** is  $a$  and the thickness of the inner coil pattern portions **61a** and **61b** is  $b$ , Equation (2) below may be satisfied. Similar to the above description, when the thickness of the outermost coil pattern portion **61c** and the thickness of the inner coil pattern portions **61a** and **61b** satisfy Equation (2) below, the final thickness  $d$  of the coil pattern formed by inducing anisotropic plating growth may be uniform, and as a result, the electronic component may have unexpectedly excellent electrical performance. Meanwhile, when a ratio between the thickness of the outermost coil pattern portion **61c** and the thickness of the inner coil pattern portions **61a** and **61b** is greater than 1.2, short-circuits may occur between the coil pattern portions due to overgrowth of the outermost coil pattern portion **61c**. Meanwhile, in Equation (2) below,  $1 < a/b < 1.8$  or  $1 < a/b < 1.2$  may be satisfied, but the range of  $a/b$  is not limited thereto:

$$1 < a/b \leq 1.8.$$

Equation (2)

As described above, the final thickness of the internal coil structure (coil pattern) formed by inducing anisotropic plating may be uniform. A difference between the sum of the thickness of the outermost coil pattern portion **61c** of the first coil pattern part **61** and a thickness of the outermost coil pattern portion **62c** of the second coil pattern part **62** grown thereon and the sum of the thickness of the inner coil pattern portion **61a** or **61b** of the first coil pattern part **61** and a thickness of an inner coil pattern portion **62a** or **62b** of the second coil pattern part **62** grown thereon may be within  $20 \mu\text{m}$ . The thickness  $d$  of each of the internal coil structures **41** and **42** may be  $200 \mu\text{m}$  to  $500 \mu\text{m}$ , and the thicknesses  $d$  of the internal coil structures **41** and **42** may be substantially equal to each other. When the final thickness of the coil pattern is uniform as described above, the electronic component may have excellent electrical performance.

As illustrated in FIG. 3, according to an exemplary embodiment, the second coil pattern part **62** may be formed by anisotropic plating, the coil pattern portions **62a**, **62b** and **62c** of the second coil pattern part **62** may be formed on upper surfaces **61T** of the coil pattern portions **61a**, **61b** and

**61c** of the first coil pattern part **61**, respectively, and side surfaces **61S** of the coil pattern portions **61a**, **61b**, and **61c** of the first coil pattern part **61** may not be covered with the second coil pattern part **62**.

For example, the upper surfaces **61T** of the coil pattern portions **61a**, **61b**, and **61c** of the first coil pattern part **61** refer to surfaces of top portions of the coil pattern portions **61a**, **61b**, and **61c** on the basis of virtual lines  $W'$  and  $W''$ , and the side surfaces **61S** of the coil pattern portions **61a**, **61b**, and **61c** of the first coil pattern part **61** refer to surfaces of side portions of the coil pattern portions **61a**, **61b**, and **61c** on the basis of the virtual lines  $W'$  and  $W''$ .

That is, the second coil pattern part **62** may not cover all of the side surfaces **61S** of the coil pattern portions **61a**, **61b** and **61c** of the first coil pattern part **61**, and accordingly, the second coil pattern part **62** may not be formed on at least a portion of the side surfaces **61S** of the coil pattern portions **61a**, **61b** and **61c** of the first coil pattern part **61**.

As described above, the coil pattern portions **62a**, **62b** and **62c** of the second coil pattern part **62** may be formed as an anisotropic plating layer which is grown on the upper surfaces **61T** of the coil pattern portions **61a**, **61b** and **61c** of the first coil pattern part **61** in the thickness direction, while inhibiting growth in the width direction. As a result, short-circuits occurring between the coil pattern portions may be prevented, and the internal coil structures **41** and **42** having a high aspect ratio (AR) may be formed. In addition, a volume of the core part **55** may be increased while direct current resistance  $R_{dc}$  is decreased, and thus, high inductance may be implemented.

The first and second coil pattern parts **61** and **62** may contain a metal having excellent electrical conductivity. For example, the first and second coil pattern parts **61** and **62** may be formed of silver (Ag), palladium (Pd), aluminum (Al), nickel (Ni), titanium (Ti), gold (Au), copper (Cu), platinum (Pt), or alloys thereof. Meanwhile, the first and second coil pattern parts **61** and **62** may be formed of the same metal. Here, the metal forming the first and second coil pattern parts **61** and **62** may be copper (Cu).

FIG. 4 is an enlarged view schematically illustrating another example of part 'A' of FIG. 2.

Referring to FIG. 4, upper surfaces **61T** of coil pattern portions **61a**, **61b** and **61c** of a first coil pattern part **61** according to another exemplary embodiment may be flat, and each of the coil pattern portions **61a**, **61b** and **61c** may have a quadrangular cross-section.

Although FIG. 3 illustrates that the upper surfaces **61T** of the coil pattern portions **61a**, **61b** and **61c** of the first coil pattern part **61** are convex and FIG. 4 illustrates that the upper surfaces **61T** of the coil pattern portions **61a**, **61b** and **61c** of the first coil pattern part **61** are flat, the shapes of the upper surfaces of the coil pattern portions are not necessarily limited thereto. That is, the cross-sectional shapes of the coil pattern portions **61a**, **61b** and **61c** of the first coil pattern part **61** may be modified within a range capable of being conceived of by a person skilled in the art.

The internal coil structures **41** and **42** may be covered with an insulating layer **30** as required. The insulating layer **30** may be formed by a method known in the art such as a screen printing method, a photo resist (PR) exposure and development method, or a spray application method. The internal coil structures **41** and **42** may be covered with the insulating layer **30**, and therefore, may not be in direct contact with a magnetic material forming the magnetic body **50**.

One end portion of the first internal coil structure **41** formed on one surface of the support member **20** may be

exposed to one end surface of the magnetic body **50** in a length (L) direction thereof, and one end portion of the second internal coil structure **42** formed on the other surface of the support member **20** may be exposed to the other end surface of the magnetic body **50** in the length (L) direction thereof.

The first and second external electrodes **81** and **82** may be formed on opposite end surfaces of the magnetic body **50** in the length L direction to be connected to the end portions of the first and second internal coil structures **41** and **42** exposed to opposite end surfaces of the magnetic body **50**, respectively.

The first and second external electrodes **81** and **82** may be formed of a metal having excellent electrical conductivity, for example, nickel (Ni), copper (Cu), tin (Sn), silver (Ag), or alloys thereof.

For example, the first and second external electrodes **81** and **82** may include a conductive resin layer and a plating layer formed on the conductive resin layer. The conductive resin layer may include at least one conductive metal selected from the group consisting of copper (Cu), nickel (Ni), and silver (Ag), and a thermosetting resin. The plating layer may include at least one selected from the group consisting of nickel (Ni), copper (Cu), and tin (Sn). For example, a nickel (Ni) layer and a tin (Sn) layer may be sequentially formed as the plating layer.

#### Method of Manufacturing Electronic Component

FIG. 5 is a flowchart schematically illustrating a method of manufacturing an electronic component according to an exemplary embodiment in the present disclosure. Referring to FIGS. 1 through 4, the method of manufacturing the electronic component is described.

First, the internal coil structures **41** and **42** may be formed on the support member **20** by plating, but the method of forming the internal coil structures **41** and **42** is not necessarily limited thereto.

As described above, the internal coil structures **41** and **42** may include the first coil pattern part **61** formed on the support member, and the second coil pattern part **62** formed on the first coil pattern part **61** (S10).

In the present exemplary embodiment, a thickness a of an outermost coil pattern portion **61c** of the first coil pattern part **61** may be thicker than a thickness b of inner coil pattern portions **61a** and **61b** thereof, such that the second coil pattern part **62** may be formed by anisotropic plating in a subsequent method, and as a result, a final thickness d of the coil pattern may be uniform. In this case, the internal coil structures **41** and **42** may be formed by plating, and the thickness a of the outermost coil pattern **61c** may be thicker than the thickness b of the inner coil pattern portions **61a** and **61b** by controlling a current density, a concentration of a plating solution, a plating rate, and the like.

Meanwhile, as described above, the insulating layer **30** covering the internal coil structures **41** and **42** may be formed to protect the internal coil structures **41** and **42**, and the insulating layer **30** may be formed by methods known in the art such as a screen printing method, a photo resist (PR) exposure and development method, or a spray application method.

Next, the magnetic body **50** may be formed by stacking magnetic sheets on and below the internal coil structures **41** and **42** formed on the support member **20**, and then compressing and hardening the magnetic sheets (S20). The magnetic sheets may be manufactured by mixing magnetic metal powder and an organic material such as a binder, a

solvent, and the like, with each other to prepare slurry, applying the slurry to carrier films to a thickness of several tens of micrometers using a doctor blade method and drying the same.

A central portion of the support member **20** may be removed by performing mechanical drilling, laser drilling, sand blasting, punching, or the like to form a hole for the core part **55**, and the hole may be filled with a magnetic material in the stacking, compressing and hardening of the magnetic sheets to form the core part **55**.

Next, the first and second external electrodes **81** and **82** may be formed on outer surfaces of the magnetic body **50** to be connected to the internal coil structures **41** and **42** exposed to the surfaces of the magnetic body **50**, respectively (S30). The external electrodes **81** and **82** may be formed by using a paste containing a metal having excellent electrical conductivity. For example, the first and second external electrodes **81** and **82** may be formed by using the conductive paste containing nickel (Ni), copper (Cu), tin (Sn), silver (Ag), or alloys thereof. In addition, a plating layer (not illustrated) may be further formed on the external electrodes **81** and **82**. In this case, the plating layer may include at least one selected from the group consisting of nickel (Ni), copper (Cu), and tin (Sn). For example, a nickel (Ni) layer and a tin (Sn) layer may be sequentially formed as the plating layer.

A description of features overlapping those of the electronic component according to the previous exemplary embodiment will be omitted.

#### Experimental Example

Table 1 below shows results obtained by measuring anisotropic plating growth of the second coil pattern part **62** formed on the first coil pattern part **61** by electroplating while changing the thickness a of the outermost coil pattern portion of the first coil pattern part and the thickness b of the inner coil pattern portions thereof.

TABLE 1

|    | Sample No. | a | b                | a - b            | a/b               | Deviation of Final Thickness | Short-Circuit Rate   |
|----|------------|---|------------------|------------------|-------------------|------------------------------|----------------------|
| 45 | *          | 1 | 50 $\mu\text{m}$ | 10 $\mu\text{m}$ | 40 $\mu\text{m}$  | 5.0                          | 60 $\mu\text{m}$ 30% |
|    | *          | 2 | 50 $\mu\text{m}$ | 20 $\mu\text{m}$ | 30 $\mu\text{m}$  | 2.5                          | 47 $\mu\text{m}$ 13% |
|    |            | 3 | 50 $\mu\text{m}$ | 30 $\mu\text{m}$ | 20 $\mu\text{m}$  | 1.7                          | 15 $\mu\text{m}$ 0%  |
|    |            | 4 | 50 $\mu\text{m}$ | 40 $\mu\text{m}$ | 10 $\mu\text{m}$  | 1.3                          | 10 $\mu\text{m}$ 0%  |
| 50 | *          | 5 | 50 $\mu\text{m}$ | 50 $\mu\text{m}$ | 0 $\mu\text{m}$   | 1.0                          | 25 $\mu\text{m}$ 10% |
|    | *          | 6 | 50 $\mu\text{m}$ | 60 $\mu\text{m}$ | -10 $\mu\text{m}$ | 0.8                          | 38 $\mu\text{m}$ 17% |
|    | *          | 7 | 50 $\mu\text{m}$ | 70 $\mu\text{m}$ | -20 $\mu\text{m}$ | 0.7                          | 58 $\mu\text{m}$ 35% |

(\* Comparative Example)

As shown in Table 1, it can be seen that when the first coil pattern part **61** satisfies Equations (1) and (2), the final thickness d of the coil pattern formed by anisotropic plating growth may be unexpectedly uniform.

Therefore, short-circuits occurring between the coil pattern portions may be unexpectedly prevented, the internal coil structures **41** and **42** may have a high aspect ratio (AR), and a volume of the core part **55** may be increased while decreasing direct current resistance Rdc, whereby high inductance may be obtained.

As set forth above, according to exemplary embodiments in the present disclosure, the thickness of a first coil pattern part may be controlled to induce anisotropic plating growth of a secondary coil pattern part, thereby providing a minia-

turized electronic component having improved electrical properties, and a method of effectively manufacturing the electronic component.

While exemplary embodiments have been shown and described above, it will be apparent to those skilled in the art that modifications and variations could be made without departing from the scope of the present disclosure as defined by the appended claims.

What is claimed is:

1. An electronic component comprising:  
a magnetic body; and  
an internal coil structure embedded in the magnetic body,  
wherein

the internal coil structure includes a first coil pattern part  
and a second coil pattern part formed on the first coil  
pattern part, and

an entire outermost coil turn of the first coil pattern part  
is thicker than an inner coil turn thereof, wherein the  
second coil pattern part has a non-uniform thickness  
such that a thickness from an uppermost surface of the  
outermost coil turn of the first coil pattern part to an  
uppermost surface of an outermost coil turn of the  
second coil pattern part is smaller than a thickness from  
an uppermost surface of the inner coil turn of the first  
coil pattern part to an uppermost surface of an inner coil  
turn of the second coil pattern part.

2. The electronic component of claim 1, wherein  $0 \mu\text{m} < a - b \leq 20 \mu\text{m}$  is satisfied, in which a is a thickness of the  
outermost coil turn of the first coil pattern part and b is a  
thickness of the inner coil turn thereof.

3. The electronic component of claim 1, wherein  $1 < a/b \leq 1.8$  is satisfied, in which a is a thickness of the outermost  
coil turn of the first coil pattern part and b is a thickness of  
the inner coil turn thereof.

4. The electronic component of claim 1, wherein a difference  
between a sum of a thickness of the outermost coil  
turn of the first coil pattern part and a thickness of an  
outermost coil turn of the second coil pattern part formed  
thereon and a sum of a thickness of the inner coil turn of the  
first coil pattern part and a thickness of an inner coil turn of  
the second coil pattern part formed thereon is within 20  $\mu\text{m}$ .

5. The electronic component of claim 1, wherein the  
second coil pattern part is formed by anisotropic plating.

6. The electronic component of claim 1, wherein the  
second coil pattern part is formed on upper surfaces of the  
coil turns of the first coil pattern part.

7. The electronic component of claim 1, wherein the  
second coil pattern part is not formed on at least a portion of  
side surfaces of the coil turns of the first coil pattern part.

8. The electronic component of claim 1, wherein the first  
and second coil pattern parts are formed of the same metal.

9. The electronic component of claim 1, wherein the  
magnetic body contains a magnetic metal powder and a  
thermosetting resin.

10. The electronic component of claim 1, wherein the  
internal coil structure comprises:

a first internal coil structure disposed on one surface of a  
support member; and  
a second internal coil structure disposed on another sur-  
face of the support member opposing the one surface  
thereof.

11. The electronic component of claim 10, wherein the  
support member has a through-hole in a central portion  
thereof, and

the through-hole is filled with a magnetic material to form  
a core part.

12. The electronic component of claim 1, further com-  
prising external electrodes disposed on outer surfaces of the  
magnetic body to be electrically connected to the internal  
coil structure.

13. The electronic component of claim 1, wherein a total  
thickness of an outermost coil turn of the first and second  
coil pattern parts is substantially the same as a total thickness  
of an inner coil turn of the first and second coil pattern parts.

14. A method of manufacturing an electronic component,  
the method comprising:

forming a first coil pattern part on a support member;  
forming a second coil pattern part on the first coil pattern  
part so as to form an internal coil structure including the  
first and second coil pattern parts; and  
forming a magnetic body by stacking magnetic sheets to  
embed the internal coil structure therein, wherein  
the forming the first coil pattern part comprises forming  
the first coil pattern part such that an entire outermost  
coil turn of the first coil pattern part is thicker than an  
inner coil turn thereof, and

the forming the second coil pattern part comprises forming  
the second coil pattern part to have a non-uniform  
thickness such that a thickness from an uppermost  
surface of the outermost coil turn of the first coil pattern  
part to an uppermost surface of an outermost coil turn  
of the second coil pattern part is smaller than a thick-  
ness from an uppermost surface of the inner coil turn of  
the first coil pattern part to an uppermost surface of an  
inner coil turn of the second coil pattern part.

15. The method of claim 14, further comprising forming  
external electrodes on outer surfaces of the magnetic body to  
be electrically connected to the internal coil structure.

16. The method of claim 14, wherein the second coil  
pattern part is formed by anisotropic plating.

17. An electronic component, comprising:  
a magnetic body; and  
an internal coil structure embedded in the magnetic body,  
wherein

the internal coil structure includes a first coil pattern part  
having a coil shape, and a second coil pattern part  
having a coil shape formed entirely and directly on the  
coil shaped first coil pattern part, and

the first coil pattern part includes a plurality of inner coil  
turns having substantially same thicknesses, and an  
outermost coil turn an entirety of which is thicker than  
the plurality of inner coil turns.

18. The electronic component of claim 17, wherein  $0 \mu\text{m} < a - b \leq 20 \mu\text{m}$  is satisfied, in which a is a thickness of the  
outermost coil turn of the first coil pattern part and b is a  
thickness of the inner coil turn thereof.

19. The electronic component of claim 17, wherein  $1 < a/b \leq 1.8$  is satisfied, in which a is a thickness of the outermost  
coil turn of the first coil pattern part and b is a thickness of  
the inner coil turn thereof.

20. The electronic component of claim 17, wherein a  
difference between a sum of a thickness of the outermost coil  
turn of the first coil pattern part and a thickness of an  
outermost coil turn of the second coil pattern part formed  
thereon and a sum of a thickness of the inner coil turn of the  
first coil pattern part and a thickness of an inner coil turn of  
the second coil pattern part formed thereon is within 20  $\mu\text{m}$ .